# EUROPEAN PATENT APPLICATION

(11) **EP 0 663 477 A1**
(43) Date of publication of application: **19.07.1995**
(21) Application number: 95300228.4
(22) Date of filing: 13.01.1995
(51) Int. Cl.: E02D 13/00, E02D 9/02

(54) **Lubricating material for extraction of temporarily buried reinforcement**

(30) Priority: 14.01.1994 JP 2723/94
(71) Applicant: NIPPON SHOKUBAI CO., LTD., Chuo-ku, Osaka-shi, Osaka-fu 541 (JP)
(72) Inventor: Okamoto, Koichi, Heights Azelea 102, Osaka-shi, Osaka-fu 535 (JP); Harada, Nobuyuki, Osaka-fu 565 (JP); Nakamura, Toshiaki, Higashinari-ku, Osaka-fu 537 (JP)
(74) Representative: Rees, David Christopher

(57) **Abstract**

A lubricating material (1) for the extraction of a temporarily buried reinforcement is proposed which excels in workability at the site of construction, allows the temporarily buried reinforcement (22) to be easily extracted and recovered from a cement layer (23), and enjoys outstanding economy. This lubricating material enables the temporary reinforcement (22) buried in the cement layer (23) to be easily separated from the cement layer (23) after the cement has been hardened. This lubricating material (1) comprises a water-absorbent polymer sheet having a water-absorbent polymer directly fixed in a substrate.

## Description

This invention relates to a lubricating material for the extraction of a temporarily buried reinforcement. More particularly, it relates to a lubricating material for the extraction of a temporarily buried reinforcement, which lubricating material is used, after a temporarily buried reinforcement such as, for example, a pile such as a steel H pile, or a steel sheet pile driven into hardening hydrate such as cement or soft ground has discharged its function, for the purpose of imparting lubricity to the interface between the temporarily buried reinforcement and the ground thereby facilitating the extraction of the temporarily buried reinforcement from the ground.

The so-called peristylar soil cement continuous wall method is counted among the methods which have been recently in popular use in the construction or the foundation of multi-story buildings, river banks, underground structures, etc. This method comprises excavating the boundary of a site for construction and filling the excavated boundary with soil cement thereby erecting a soil cement wall intended to hold back the hydraulic pressure of soil. Since this wall of soil cement is deficient in strength as compared with ordinary concrete, such temporary reinforcements as steel H piles are incorporated in the soil cement layer. Also in the work of reinforcing an excavation, piles like steel H piles are buried in a cementitious substance and a concrete wall is erected as supported by the steel H pile-reinforced cementitious substance. The temporary reinforcements like steel H piles which have been driven into the cement layer have too high adhesiveness to the hardened cement to be easily extracted from the hardened cement. Thus, it has been customary for these reinforcements to be left buried in the cement after the work of reinforcement has been completed.

Generally, the steel materials which have been used as temporarily buried reinforcements are not always found to be necessary from the standpoint of strength after the cement has been hardened. When the used steel materials which have played their part as temporarily buried reinforcements in the work are extracted from the hardened cement layer and put to use again, they ought to contribute immensely to economize the work. This practice of reclaiming the used steel materials has the advantage of facilitating such secondary works as the expansion and the remodeling of existing buildings and the construction of sewerage systems and water supply systems.

For facilitating the extraction of such steel materials from the hardened cement, JP-A-58-104,058 proposes a method which comprises applying an organic substance containing wax or sugar to the surface of a given temporarily buried reinforcement and putting the coated reinforcement to use. This method, when using wax in the organic coating substance, requires the wax to be melted by heating and consequently betrays deficiency in quickness and efficiency of the work to be involved. The method, when using sugar instead, is not necessarily a wise choice because the effect of preventing the hardening of cement possibly expands to the inner part of the mass of cement and eventually impairs the strength of the cement mass.

Recently, several methods have been proposed which have in common the procedure comprising the steps of preparing a temporary reinforcement having a water-absorbent polymer deposited on the surface thereof, driving the coated temporary reinforcement into a cement layer thereby enabling the water-absorbent polymer layer swelled by the absorption of cement water to interpose a gap between the reinforcement and the cement layer, and allowing the swelled water-absorbent polymer gel to function as a lubricating material during the extraction of the temporarily buried reinforcement thereby enabling the reinforcement to be easily extracted and recovered.

JP-B-04-44,045, for example, discloses a method which facilitates the extraction of a temporarily buried reinforcement by preparatorily applying to the entire surface of this reinforcement an absorbent lubricating tape having an water-absorbent polymer fixed thereon with such a rewetting binder as starch paste.

This method, however, is not easily adaptable for actual use particularly in the work at a site of construction because the work of applying the tape to the entire surface of the temporary reinforcement is extremely troublesome. Further, since the water-absorbent polymer is fixed with the rewetting binder such as starch paste and consequently the force of adhesion of the water-absorbent polymer to the substrate of the tape is so weak that the water-absorbent polymer possibly peels off the reinforcement while the reinforcement is being used, the water-absorbent polymer layer cannot be easily installed at the prescribed position and the water-absorbent polymer cannot be used as a lubricating material. An idea of using the binder in an increased amount for the purpose of curbing the accidental separation of the water-absorbent polymer is conceivable. The increase in the amount of the binder to be used, however, imposes a restriction on the degree to which the water-absorbent polymer swells and consequently prevents the water-absorbent polymer from absorbing water amply and compels it to manifest only an insufficient lubricating effect during the extraction of the temporarily buried reinforcement. JP-A-01-58,715 discloses a method which resides in directly coating to a core member a surface treating agent which is composed of a water-absorbent polymer and an extender at a prescribed weight ratio. To date, this method has not produced a satisfactory result because it still entails a troublesome work and has not perfectly solved the two problems, i.e. accidental separation of the water-absorbent polymer and the degradation of the capacity for absorption by the extender. Moreover, this method necessitates the addition of a solvent for the dispersion of an extender in the coating material with a sacrifice of the safety of the working environment.

In order that the temporarily buried reinforcements according to the conventional methods may be extracted and put to use again, the temporarily buried reinforcements which have been extracted from the cement layer must be stripped of either the water-absorbent polymer or the adhesive agent still adhering to their surfaces and then coated anew with a lubricating tape or a surface treating agent. Thus, even from the standpoint of the reuse, the conventional methods prove to be troublesome and uneconomical.

Further, there are cases in which the temporarily buried reinforcements are left standing in the cement layer after the cement is hardened for a long time even exceeding one half year before they are extracted from the hardened cement layer. Thus, the possibility arises that the water-absorbent polymer, during the protracted standing of the buried reinforcements, will be gradually shrunken under the influence of the polyvalent metal salt contained in the cement water (breeding water) and will fail to function as a lubricating material during the extraction of the buried reinforcements.

An object of this invention, therefore, is to provide a novel lubricating agent for the extraction of temporarily buried reinforcements.

Another object of this invention is to provide a lubricating material for the extraction of temporarily buried reinforcement, which lubricating material excels in applicability to a substrate at the site of construction, allows the temporarily buried reinforcements using it to be easily extracted from the cement layer, recovered, and put to use again after the construction is completed, and proves to be highly economical.

The objects mentioned above are accomplished by a lubricating material for the extraction of temporarily buried reinforcements, which lubricating material is characterized by being provided with a water-absorbent polymer sheet layer having a water-absorbent polymer directly deposited fast on a substrate.

This invention further concerns the lubricating material for the extraction of the temporarily buried reinforcements, wherein the water-absorbent polymer has been obtained by polymerizing a water-soluble ethylenically unsaturated monomer capable of being converted by polymerization into a water-absorbent polymer on the substrate. This invention further concerns the lubricating material for the extraction of the temporarily buried reinforcements, wherein the substrate is a porous material. This invention further concerns the lubricating material for the extraction of the temporarily buried reinforcements, wherein the amount of the water-absorbent polymer is in the range of from 10 to 1000 parts by weight, based on 100 parts by weight of the substrate. This invention further concerns the lubricating material for the extraction of the temporarily buried reinforcements, wherein the porous material is a fibrous material or sponge. This invention further concerns the lubricating material for the extraction of the temporarily buried reinforcements, wherein a thickness of said lubricating material is in the range of from 10 to 1000 µm. This invention further concerns the lubricating material for the extraction of the temporarily buried reinforcements, wherein the water-absorbent polymer has been obtained by polymerizing a monomer having as a main component thereof at least one water-soluble ethylenically unsaturated monomer selected from the group consisting of (meth)acrylic acid, (meth)acrylic acid salts, sulfonic acid group-containing (meth)acrylic esters and salts thereof, and 2-(meth)acrylamide-2-methylpropane sulfonic acid and salts thereof. This invention further concerns the lubricating material for the extraction of the temporarily buried reinforcements, wherein the water-absorbent polymer contains a sulfonic acid group obtained by polymerizing a water-soluble unsaturated monomer containing a water-soluble ethylenically unsaturated monomer. This invention further concerns the lubricating material for the extraction of the temporarily buried reinforcements, wherein the water-soluble ethylenically unsaturated monomer contains a cross-linking agent in an amount in the range of from 0.001 to 10 mol%, based on the amount of the monomer. This invention further concerns the lubricating material for the extraction of the temporarily buried reinforcements, which is further provided on one side of the water-absorbent polymer sheet layer with a water-impermeable layer. This invention further concerns the lubricating material for the extraction of the temporarily buried reinforcements, wherein a thickness of the water-impermeable layer is in the range of 1 to 1000 µm. This invention further concerns the lubricating material for the extraction of the temporarily buried reinforcements, which is in the shape of a bag or a tube. This invention further concerns the lubricating material for the extraction of the temporarily buried reinforcements, which is further provided with a water-impemeable layer on the inner side of the water-absorbent polymer layer in the shape of a bag or a tube. This invention further concerns the lubricating material for the extraction of the temporarily buried reinforcements, which is further provided at the opening part of the bag or the tube with a hanger.

The lubricating material of this invention for the extraction of the temporarily buried reinforcements is used to cover the surface of the temporary reinforcement such as the pile of an steel H pile or the steel sheet pile of a flat steel plate which is destined to hold back the hardening hydrate such as the soft ground of silt or sludge or the cement before the reinforcement is placed in the silt or the cement. After the work of construction associated with the silt or the cement is completed, the temporarily buried reinforcement is no longer useful and is extracted from the silt or the cement. The extraction of the temporarily buried reinforcement, therefore, is facilitated by the fact that the lubricating material is used on the steel H pile or the steel sheet pile.

The lubricating material of this invention for the extraction of the temporarily buried reinforcements permits lasting preclusion of the accidental separation of the polymer, enjoys a high lubricating property, facilitates saliently the extraction and recovery of the buried reinforcements from the cement layer, and contributes to economize the use of the temporary reinforcements. It also contributes to improve the efficiency of the work of handling at the site of construction, the secondary work, or the work of recovering the buried reinforcements and putting it to use again.

The lubricating material for the extraction of the temporarily buried reinforcements of this invention, therefore, can be used as a material for facilitating the recovery of such temporary reinforcements as the steel H piles and the steel sheet piles from the cement layers and the soft grounds which are formed in various foundation works for multi-story buildings, expressways, bridges, river banks, lakes, waterfronts, and ports and harbors, various underground works for underground cities, subways, ground surfaces, sewerages, city water pipes, gas pipes, and electric wirings, and works for excavation.

When the lubricating material for the extraction of temporary reinforcements is formed in the shape of a bag or a tube, it facilitates the work of placing such temporary reinforcements as the steel H piles and the steel sheet piles. When a layer impermeable to water is provided on one side of the water-absorbent polymer or inside the bag or the tube of the lubricating material, it keeps the cement milk from permeating the buried reinforcement and prevents the buried reinforcement from gathering stain.

The invention may be carried into practice in various ways and some embodiments will now be described by way of example with reference to the accompanying drawings, in which:-

Fig. 1 is a cross section illustrating one embodiment of the lubricating material of this invention for the extraction of temporarily buried reinforcements.

Fig. 2 is a cross section illustrating another embodiment of the lubricating material of this invention for the extraction of temporarily buried reinforcements.

Fig. 3 is a diagram illustrating the manner in which an steel H pile is in the process of being inserted into a lubricating material for the extraction of a temporary reinforcement fabricated in the shape of a bellows and posed for insertion into a mass of cement.

Fig. 4 is a diagram illustrating one embodiment of the disposition in a steel H pile of the lubricating material of this invention for the extraction of a temporarily buried reinforcement.

Fig. 5 is a diagram illustrating another embodiment of the disposition in a steel H pile of the lubricating material of this invention for the extraction of a temporarily buried reinforcement.

Fig. 6 is a diagram illustrating still another embodiment of the disposition in a steel H pile of the lubricating material of this invention for the extraction of a temporarily buried reinforcement.

Fig. 7 is a diagram illustrating yet another embodiment of the disposition in a steel H pile of the lubricating material of this invention for the extraction of a temporarily buried reinforcement.

Fig. 8 is a diagram illustrating the state in which the lubricating material for the extraction of temporary reinforcement has been fixed on a steel H pile.

Now, this invention will be described more specifically below with reference to the annexed drawings.

As illustrated in Fig. 1, a lubricating material 1 of this invention which is provided with a water-absorbent polymer sheet layer and adapted for the extraction of a temporarily buried reinforcement is furnished with a water-absorbent polymer sheet layer 3 having a water-absorbent polymer directly deposited fast on a substrate 2 without use of a binder. Owing to the fact that no binder is used, the water-absorbent polymer layer can be interposed between the temporary reinforcement and the cement layer without either sacrificing the absorbing property inherent in the water-absorbent polymer or entailing accidental separation of the water-absorbent polymer and can be used as a lubricating material for the extraction of the temporarily buried reinforcement.

Fig. 2 illustrates another preferred embodiment of this invention. It is a lubricating material 11 for the extraction of a temporarily buried reinforcement having a water-absorbent polymer sheet layer 13 formed on a substrate 12 without use of a binder and having a layer 14 impermeable to water deposited on one side of the water-absorbent polymer sheet layer 13.

The water-absorbent polymer which is advantageously used in the present invention is obtained by polymerizing a water-soluble ethylenically unsaturated monomer having as a main component thereof acrylic acid, an acrylate, or a sulfonic acid group-containing (meth)acrylic ester or an acid thereof and optionally incorporating therein a crosslinking agent and consequently adapted to swell by absorbing from 10 to 1000 times its own weight of water. Although a thickness of the substrate is not limited, it is generally in the range of 0.01 to 10mm, and a basis weight thereof is in the range of 10 to 500g/m².

As other typical example of the water-absorbent polymer which is mentioned above, cross-linked polyethylene oxide, cross-linked polyvinylpyrrolidone, sulfonated crosslinked polystyrene, cross-linked polyvinyl pyridine, saponified starch-poly(meth)-acrylonitrile graft copolymer, cross-linked starch-poly(meth)-acrylic acid (acrylate) graft copolymer, the reaction product of polyvinyl alcohol with maleic anhydride (salt), cross-linked polyvinyl alcohol sulfonates, and polyvinyl alcohol-acrylic acid graft copolymer may be cited.

As typical examples of the substrate to be used for this invention, hydrophilic or hydrophobic porous materials such as woven fabrics, non-woven fabrics, knit fabrics, paper, and sponge may be cited. The fact that the substrate contains voids therein is at an advantage in enabling the water-absorbent polymer to acquire empty spaces available for the purpose of swelling and ensuring effective contact between the cement water and the water-absorbent polymer. As typical examples of the raw material for use in the substrate, hydrophilic fibers such as of wood pulp, cotton, wool, rayon, acetate, and vinylon and hydrophobic fibers such as of polyester, polyacrylonitrile, nylon, polypropylene, polyethylene, polyurethane, polyvinyl chloride, glass wool, and rock wool may be cited where the substrate is a fibrous substrate. Where the substrate is a spongy substance, polyacetal, polyurethane, cellulose, and phenol resin may be cited as concrete examples of the raw material usable therefor. From the viewpoint of the workability, flexibility, and economy of the lubricating material to be produced and used for the extraction of the temporarily buried reinforcement, it is particularly desirable to use for the substrate the non-woven fabric of hydrophobic fibers of polyester or polypropylene among other raw materials mentioned above.

For use in the present invention, the amount of the water-absorbent polymer is in the range of from 10 to 1000 parts by weight, preferably from 80 to 500 parts by weight, based on 100 parts by weight of the substrate. If the amount of the water-absorbent polymer is less than 10 parts by weight, the disadvantage will arise that the water-absorbent polymer manifests an unduly small lubricating effect for the sake of the extraction of the temporarily buried reinforcement. Conversely, if this amount exceeds 1000 parts by weight, the disadvantage will arise that the produced water-absorbent polymer sheet acquires unduly low flexibility and suffers from deficiency in workability.

The water-absorbent polymer sheet which has the water-absorbent polymer directly deposited fast on the substrate is obtained by a) a method which comprises directly spraying on the substrate the water-absorbent polymer softened in advance with water and optionally drying the applied layer of the water-absorbent polymer, B) a method which comprises applying to the substrate a water-soluble polymer capable of being converted by cross-linking into the water-absorbent polymer and then cross-linking the applied layer of the water-soluble polymer, or C) a method which comprises applying to the substrate a monomer capable of being converted by polymerization into the water-absorbent polymer and then polymerizing the applied layer of the monomer, for example. The method to be adopted for this production of the water-absorbent polymer sheet has no particular restriction except for the requirement that it be capable of directly depositing the water-absorbent polymer fast on the substrate through no medium of a binder.

Among other methods mentioned above, the method which comprises applying to the substrate a monomer capable of being converted by polymerization into the water-absorbent polymer and subsequently polymerizing the applied layer of the monomer proves to be particularly desirable from the viewpoint of the convenience and the economy of manufacture and the durability of the produced water-absorbent polymer sheet. By this method, the water-absorbent polymer sheet which has the water-absorbent polymer directly deposited fast on the substrate can be easily and conveniently obtained.

As typical examples of the monomer which can be converted by polymerization into the water-absorbent polymer, acrylic acid and methacrylic acid and alkali metal salts and ammonium salts thereof; 2-(meth)acryloylethanesulfonic acid, 2-(meth)acryloyl propanesulfonic acid, 2-(meth)acrylamide-2-methylpropanesulfonic acid, vinylsulfonic acid, (meth)allylsulfonic acid and alkali metal salts and ammonium salts thereof; (meth)acrylamide, N,N'-dimethylaminoethyl(meth)acrylates and quaternization products thereof; and hydroxyalkyl(meth)acrylates and polyalkylene glycol (meth)acrylates may be cited. These monomers may be used either singly or in the form of a mixture of two or more members.

From the viewpoint of the ability of the lubricating material to swell by absorbing the cement water, such sulfonic acid group-containing water-soluble ethylenically unsaturated monomers as 2-(meth)acryloylethanesulfonic acid, 2-(meth)-acryloylpropanesulfonic acid, 2-(meth)acrylamide-2-methyl propanesulfonic acid, vinylsulfonic acid, (meth)allylsulfonic acid, and alkali metal salts and ammonium salts thereof prove to be particularly preferable. The lubricating material of this invention for the extraction of a temporarily buried reinforcement which is formed of the water-absorbent polymer sheet obtained by depositing the sulfonic acid group-containing water-soluble ethylenically unsaturated monomer on the substrate and consequently polymerizing or cross-linking the applied layer of the monomer succumbs only sparingly to the influence of the polyvalent metal salt such as calcium salt contained in the cement water and pH, and, therefore, enjoys a stable ability to swell by absorbing the cement water, and further facilitates the extraction of a temporarily buried reinforcement.

The monomer mentioned above may have incorporated therein a polyfunctional water-soluble ethylenically unsaturated monomer as a cross-linking agent. As typical examples of the monomer which is usable as the cross-linking agent, divinyl benzene, ethylene glycol di(meth)acrylate, diethylene glycol di(meth)acrylate, triethylene glycol di(meth)acrylate, propylene glycol di(meth)acrylate, polyethylene glycol di(meth)acrylate, trimethylol propane tri(meth)acrylate, pentaerythritol (meth)acrylate, pentaerythritol di(meth)acrylate, N,N-methylenebisacrylamide, triallyl isocyanurate, and trimethylol propane diallyl ether may be cited. The use of this cross-linking agent contributes to improve the durability and the shape-retaining property of the produced lubricating material. Though the amount of the crosslinking agent to be used may be suitably selected in accordance with the kind of the monomer and the conditions for the polymerization of this monomer, it is generally in the range of from 0.001 to 10 mol%, preferably from 0.01 to 5 mol% (based on the amount of the monomer).

The method for effecting the deposition of the monomer mentioned above on the substrate has no particular restriction. This deposition of the monomer on the substrate can be attained, for example, by preparing the monomer in the form of an aqueous solution, depositing the aqueous solution on the substrate by printing, spraying, or impregnating the substrate with the monomer solution followed by squeezing off to a specified amount. The monomer which has been deposited on the substrate as described above is polymerized by the known technique to accomplish the direct deposition of the water-absorbent polymer on the substrate. This polymerization can be effected by any of the known methods which resort to the actions of heat, light, electron beam, ultraviolet light, etc. The aqueous solution of the monomer mentioned above may additionally contain therein a water-soluble radical polymerization initiator such as persulfate, a water-soluble amino compound, etc. or other additives as occasion demands.

The lubricating material of this invention for the extraction of a temporarily buried reinforcement which is formed as described above has a thickness in the range of from 10 to 1000 µm, preferably from 20 to 500 µm. If this thickness is less than 10 µm, the lubricating material will be deficient not only in mechanical strength but also in the ability to absorb water and the lubricity necessary for the extraction of the temporarily buried reinforcement. Conversely, if this thickness exceeds 1000 µm, the lubricating material sometimes lacks flexibility and it is sometimes difficult to attach the lubricating material on the surface of the temporarily buried rein for cement.

The lubricating material of this invention which is provided with the water-absorbent polymer sheet layer obtainable as described above and is used for the extraction of a temporarily buried reinforcement has the water-absorbent polymer directly deposited fast on the substrate as described above. During the insertion of the temporary reinforcement into the cement layer, the swelling of the water-absorbent polymer with the cement water, or the extraction of the buried reinforcement from the hardened cement layer, therefore, the accidental separation of the water-absorbent polymer occurs very rarely. Thus, the water-absorbent polymer is deposited uniformly throughout the entire surface of the temporarily buried reinforcement. The lubricating material of this invention, therefore, manifests extremely high lubricity during the extraction of the temporarily buried reinforcement.

Further, the lubricating material of this invention for the extraction of the temporarily buried reinforcement is allowed to exhibit a high swelling property because it avoids using such a binder as impedes the water-absorbent polymer from swelling by absorption in the fast deposition of the water-absorbent polymer on the substrate. The use of the lubricating material of this invention, therefore, allows a large gap to be formed between the temporarily buried reinforcement and the cement layer and aids in decreasing the frictional resistance generated during the extraction of the temporarily buried reinforcement.

When the water-absorbent polymer sheet layer mentioned above is provided on one side thereof with a water-impermeable layer, the lubricating material facilitates the extraction of the temporarily buried reinforcement to a greater extent.

The material for the water-impermeable layer has no particular restriction except for the requirement that it be impermeable to water and capable of being applied fast to the water-absorbent polymer sheet layer mentioned above. As concrete examples of the material satisfying this requirement, hydrophobic resinous films and boards such as of polyester, polyacrylonitrile, nylon, polypropylene, polyethylene, polyvinyl chloride, and polyurethane; aluminum foil; and metallic films such as of aluminum may be cited. Among other materials mentioned above, the resinous film layers such as of polyester, polyacrylonitrile, nylon, polypropylene, polyethylene, polyvinyl chloride, and polyurethane prove to be particularly desirable from the viewpoint of the flexibility, workability, and economy of the water-absorbent polymer sheet provided with the layer impermeable to water. The water-impermeable layer has a thickness in the range of from 1 to 1000 µm, preferably from 10 to 500 µm.

The fast attachment of the material impermeable to water to one side of the water-absorbent polymer sheet layer mentioned above can be attained by a method which effects the attachment through the medium of a binding agent such as a tackiness agent or an adhesive agent or a method which attains the attachment by preparing the material under consideration in a thermally molten state, extruding the thermally molten material, and applying the extruded molten material to the one side, for example. The method which attains the application by the extrusion of the thermally molten material proves to be preferable from the viewpoint of the efficiency of manufacture, flexibility, workability, and economy of the lubricating material.

When the lubricating material which is provided with the water-impermeable layer is to be deposited on the surface of a given temporary reinforcement, it ought to be attached to the surface in such a manner that the water-impermeable layer may fall on the temporary reinforcement side and the water-absorbent polymer layer may fall on the cement layer side. The water-impermeable layer which is used in the lubricating material as deposited on one side of the water-absorbent polymer sheet layer prevents the cement still in a fluid state from passing to the temporary reinforcement side, ensures perfect separation of the cement layer from the temporary reinforcement, and allows the temporarily buried reinforcement to be easily extracted and recovered. The reinforcement so recovered can be put to use again in its unmodified form because neither cement adheres to nor rust forms on the surface of the recovered reinforcement.

For the purpose of further enhancing the lubricity of the temporarily buried reinforcement or the resistance of the reinforcement to rusting and corrosion, a lubricant such as wax or a rust preventive may be preparatorily applied to the surface of the temporary reinforcement.

The lubricating material of this invention for the extraction of the temporarily buried reinforcement is disposed on the surface of a given temporary reinforcement before this temporary reinforcement is driven into a hardening hydrate such as cement. The disposition of the lubricating material on the surface of the temporary reinforcement may be attained by such a method as wrapping the temporary reinforcement with the lubricating material or nipping it between the opposed pieces of the lubricating material, for example. The lubricating material may be fastened to the temporary reinforcement with bolts or attached fast thereto with a varying adhesive agent. From the viewpoint of the workability at the site of construction, the method of fabricating the lubricating material for the extraction of the temporarily buried reinforcement in the form of a bag and wrapping a given temporary reinforcement with the bag proves to be particularly preferable. The lubricating material thus fabricated in the form of a bag can be easily disposed on the surface of such a large and heavy temporary reinforcement as a steel H pile. The lubricating material which has been fabricated in the form of a bag is preferable further to be corrugated. The corrugated lubricating material is at an advantage in acquiring a compact shape, avoiding to occupy a large space at the site of construction, and ensuring easy disposition on the temporary reinforcement.

The lubricating material for the extraction of the temporarily buried reinforcement may be disposed on a given temporary reinforcement in advance of the transportation of the temporary reinforcement to the site of construction. Preferably, it is disposed on the temporary reinforcement at the site of construction in advance of the placement of the temporary reinforcement in the cement. The method to be adopted for the disposition of the lubricating material on the temporary reinforcement at the site of construction has no particular restriction. Figs. 3 to 5 depict typical examples of the method available for this purpose. Fig. 3 represents the method which comprises setting a corrugated lubricating material 21 for the extraction of a temporarily buried reinforcement on a supporting base 25 and inserting a steel H pile 22 downward (in the direction of A) into the corrugated bag of the lubricating material 21 and, at the same time, driving the steel H pile into a soil cement 23 which fills a hole excavated in the ground. The corrugated bag of the lubricating material 21 is lined, when necessary, with a polypropylene water-impermeable layer (not shown). The bag has the bottom thereof heat sealed so as to prevent the cement 23 in a fluid state to permeate the lubricating material 21 and contact the steel H pile 22. Since the lubricating material 21 for the extraction of the temporarily buried reinforcement illustrated in Fig. 3 is fabricated in the shape of a corrugated bag, it avoids occupying an unduly large space and can be disposed on the surface of the steel H pile 22 by a simple work of inserting the H bar 22 downward into the bag.

Fig. 4 represents the method which comprises slipping the corrugated lubricating material 21 for the extraction of the temporarily buried reinforcement on one end of the steel H pile 22, then lifting the steel H pile 22 as with a crane 27, and subsequently causing the lubricating material 21 to be pulled down with a cord 28 handled by a human being 29 thereby completing the disposition of the lubricating material 21 on the surface of the steel H pile 22. For the purpose of preventing the cement in a fluid state from contacting the steel H pile 22, the lubricating material 21 for the extraction of the temporarily buried reinforcement may be lined with a layer impermeable to water or the bag of the lubricating material 21 may have the lower end thereof heat sealed.

Fig. 5 represents the method which comprises keeping the steel H pile 22 suspended as by a crane 27 and lifting the bag-shaped lubricating material 21 with the cord 28 through the medium of a pulley 30 until the steel H pile 22 is completely covered with the bag. The bag, when necessary for preventing the cement in a fluid state from contacting the steel H pile 22, may be lined with a water impermeable layer (not shown). The cord 28 is attached at one end thereof to the upper part of the bag and passed around the pulley 30 fixed to the leading end of the crane 27. It is pulled up with the force of the human being 29 until the bag completely envelopes the steel H pile 22. After the bag of the lubricating material 21 has been pulled up completely, it is cut in a suitable length and the lower cut end of the bag is sealed with an adhesive agent or by heat sealing so as to prevent the cement in a fluid state from entering the bag through the lower cut end. Alternatively, the lower cut end of the bag may be tied as with a cord to preclude the otherwise possible invasion of the bag interior by the fluid cement. Also by this method, the disposition of the lubricating material 21 for the extraction of the temporarily buried reinforcement on the surface of the steel H pile 22 can be easily attained. It should be noted that they are not the only methods that are available for the disposition of the lubricating material for the extraction of the temporarily buried reinforcement on the surface of the temporary reinforcement.

Fig. 6 represents another example of the method available for the attachment of the lubricating material 21 for the extraction of the temporarily buried reinforcement to the steel H pile 22 which is a temporary reinforcement. This method comprises setting the lubricating material 21 for the extraction of the temporarily buried reinforcement in place as posed in the shape of a folded bag or tube, inserting the steel H pile 22 into an opening end 31 of the bag or tube, and giving a pull at the cord 28 thereby lifting the opening end 3 until the bag or tube wraps the steel H pile 22 completely.

Fig. 7 and Fig. 8 represent other examples of the method available for the attachment under consideration. These methods have in common the procedure which comprises attaching a hanger 33 through the medium of a cord 32 to the opening end 31 of the lubricating material 21 for the extraction of the temporarily buried reinforcement fabricated in the shape of a bag or a tube, inserting the steel H pile 22 into the opening end 31 of the lubricating material 21, giving a pull at the cord 28 thereby lifting the opening end 31 together with the hanger 33 and causing the lubricating material 21 for the extraction of the temporarily buried reinforcement to ascend along the lateral face of the steel H pile 22, and discontinuing the pull of the cord 28 after the opening end 31 reaches a level slightly above the upper end of the steel H pile 22 thereby allowing the hanger 33 to fall and settle on the upper end of the steel H pile 22. As a result, the necessity for particularly fixing the lubricating material 11 during the subsequent work of insertion into the cement can be obviated.

The lubricating material for the extraction of the temporarily buried reinforcement can be fabricated in the shape of a bag or a tube as by means of heat sealing, adhesion, sewing, or connection.

Since the water-absorbent polymer sheet layer which is provided for the lubricating material of this invention for the extraction of the temporarily buried reinforcement has the water-absorbent polymer directly deposited fast on the substrate, it rarely suffers from accidental separation of the water-absorbent polymer during the insertion of the reinforcement into the cement layer, the extraction of the reinforcement from the cement layer, or the swelling of the water-absorbent polymer sheet layer with the cement water. Thus the water-absorbent polymer is disposed uniformly throughout the entire surface of the reinforcement and allowed to manifest extremely high lubricity during the extraction of the reinforcement. Further, since the water-absorbent polymer sheet layer uses no binder, the water-absorbent polymer encounters no obstruction in swelling with the absorbed cement water and allows the interposition of a large gap between the reinforcement and the cement layer. Thus, the use of the lubricating material of this invention for the extraction of the temporarily buried reinforcement permits a decrease in the frictional resistance offered during the extraction of the temporarily buried reinforcement and facilitates the extraction and recovery of the reinforcement to a great extent.

The lubricating material of this invention for the extraction of the temporarily buried reinforcement features thinness and flexibility because the water-absorbent polymer layer provided therefor has a small thickness and has the water-absorbent polymer directly deposited fast on the substrate formed of flexible fibers or non-woven fabric. Thus, the disposition of the lubricating material of this invention for the extraction of the temporarily buried reinforcement on the surface of a reinforcement destined to be driven into the cement layer can be attained by a simple work of nipping or wrapping. As a result, the lubricating material enjoys high workability and great ease of handling. Further, it can be easily fabricated in the shape of a bag or combined with other material by means of heat sealing, sewing, and connection. When the lubricating material of this invention for the extraction of the temporarily buried reinforcement is produced in the shape of a bag from the beginning, it enjoys a further improvement in workability as evinced by the fact that the disposition thereof on a given reinforcement is accomplished simply by inserting this reinforcement in the bag.

By forming a water-impermeable layer on one side of the water-absorbent polymer sheet layer and causing this water-impermeable layer to fall on the reinforcement side when the lubricating material is put to use, the passage of the fluid cement to the reinforcement side can be prevented, the perfect separation of the cement layer and the reinforcement can be obtained, and the extraction of the reinforcement can be facilitated to a great extent. In contrast to the conventional lubricating material which suffers the temporarily buried reinforcement to be extracted in a state having the water-absorbent polymer or the binding agent incorporated therein still attached to the surface thereof, the lubricating material of this invention for the extraction of the temporarily buried reinforcement which is provided with the water-absorbent polymer sheet layer allows the temporarily buried reinforcement to be extracted and recovered exclusively because the lubricating material does not adhere to the reinforcement during the extraction of this reinforcement. For this reason, the lubricating material for the extraction of the temporarily buried reinforcement which has been used once does not need to be removed elaborately from the surface of the extracted reinforcement but allows very convenient reuse of the extracted reinforcement. The extracted reinforcement can be put to use again with the surface thereof in a state neither smeared with cement or soil nor defiled with rust.

When the water-absorbent polymer directly deposited fast on the substrate is a polymer containing a sulfonic acid group, it is only sparingly susceptible of the influence of the calcium salt contained in the cement water and, therefore, manifests stably a prominent ability to swell with the cement water, functions ideally as a lubricating material, and further enhances the ease of extraction of the temporarily buried reinforcement.

Now, this invention will be described more specifically below with reference to working examples. It should be remarked that this invention is not limited to these working examples.

### Example 1

An aqueous 40 wt% monomer solution was produced by preparing an aqueous solution of sodium acrylate having a 75% portion thereof neutralized with sodium hydroxide and dissolving 0.12 mol% of N,N-methylenebisacrylamide (based on the amount of the sodium acrylate monomer) and 1.0 g/mol of sodium persulfate (based on the amount of the sodium acrylate monomer) in the aqueous sodium acrylate solution. A non-woven fabric made of polypropylene and having a basis weight of 25 g/m² was immersed in the aqueous monomer solution and impregnated with this solution and then wrung with rollers to remove excess aqueous monomer solution. The impregnated non-woven fabric was heated to effect radical polymerization of the monomer solution in the fabric and obtain a water-absorbent polymer sheet (1) having a water-absorbent polymer directly fixed at a ratio of 40 g/m² in the fabric as a substrate. This water-absorbent polymer sheet (1) was labeled "a lubricating material (1) of this invention for the extraction of a temporarily buried reinforcement." It had a thickness of 200 µm.

A planar iron sheet 150 mm in height and 70 mm in width was wrapped with the lubricating material (1) of this invention for the extraction of a temporarily buried reinforcement and placed in a container filled with cement milk obtained by blending cement, water, bentonite, and earth. The planar iron sheet wrapped with the lubricating material (1) of this invention for the extraction of the temporarily buried reinforcement, after three months' standing in the container, was tested for the strength required for the extraction thereof from the cement.

The planar iron sheet wrapped with the lubricating material (1) could be easily extracted with a strength of 15 g/cm². The lubricating material (1) for the extraction of the temporarily buried reinforcement could be readied for use by a simple work of wrapping the planar iron sheet therewith. Thus, it enjoyed high workability and great ease of handling.

### Example 2

An aqueous 45 wt% monomer solution was produced by preparing an aqueous solution of the potassium salt of 2-acryloylpropanesulfonic acid and dissolving 0.1 mol% of N,N-methylenebisacrylamide (based on the amount of the potassium salt monomer of 2-acryloylpropanesulfonic acid) and 1.0 g/mol of sodium persulfate (based on the amount of the potassium salt monomer of 2-acryloylpropanesulfonic acid). A non-woven fabric made of polyester and having a basis weight of 30 g/m² was immersed in the aqueous monomer solution and impregnated with this solution and then wrung with rollers to remove excess aqueous monomer solution. The impregnated non-woven fabric was heated to effect radical polymerization of the monomer solution in the fabric and obtain a water-absorbent polymer sheet (2) having a water-absorbent polymer containing a sulfonic acid group directly fixed at a ratio of 70 g/m² in the fabric as a substrate. This water-absorbent polymer sheet (2) was labeled "a lubricating material (2) of this invention for the extraction of a temporarily buried reinforcement." It had a thickness of 250 µm.

A planar iron sheet 150 mm in height and 70 mm in width was wrapped with the lubricating material (2) of this invention for the extraction of a temporarily buried reinforcement and placed in a container filled with cement milk obtained by blending cement, water, bentonite, and earth. The planar iron sheet wrapped with the lubricating material (1) of this invention for the extraction of the temporarily buried reinforcement, after three months' standing in the container, was tested for the strength required for the extraction thereof from the cement.

The planar iron sheet wrapped with the lubricating material (2) could be easily extracted with a strength of 11 g/cm². The lubricating material (2) for the extraction of the temporarily buried reinforcement manifested an ideal ability to swell with water stably for a long time. It could be readied for use by a simple work of wrapping the planar iron sheet therewith. Thus, it enjoyed high workability and great ease of handling.

### Example 3

A lubricating material (3) of this invention for the extraction of a temporarily buried reinforcement was produced by melt extruding polypropylene and applying the extruded molten polymer to one side of the water-absorbent polymer sheet (1) obtained in Example 1 thereby providing a water-impermeable polypropylene layer 30 µm in thickness on one side of the water-absorbent polymer sheet. This lubricating material (3) had a thickness of 250 µm.

Then, the lubricating material (3) for the extraction of the temporarily buried reinforcement was heat sealed in the shape of a bag with the polypropylene layer falling on the inner side of the bag.

A planar iron sheet 150 mm in height and 70 mm in width was inserted in the bag of the lubricating material (3) for the extraction of the temporarily buried reinforcement and then placed in a container filled with cement milk obtained by blending cement, water, bentonite, and earth. The planar iron sheet inserted in the lubricating material (3) of this invention for the extraction of the temporarily buried reinforcement, after 3 months' standing in the container, was tested for the strength required for the extraction thereof from the cement.

This planar iron sheet could be easily extracted with a force of 10 g/cm². Further, the lubricating material (3) for the extraction of the temporarily buried reinforcement could be readied for use by a simple work of inserting the planar iron sheet in the bag of the lubricating material (3). Thus, it enjoyed high workability and great ease of handling. When the planar iron sheet was extracted from the cement, it did not suffer the used lubricating material (3) to persist on the surface of the extracted planar iron sheet. The planar iron sheet thus extracted was in such a state that it could be directly put to use again without any modification.

### Control 1

A mixed liquid obtained by mixing 100 parts of starch paste with 20 parts of a water-absorbent polymer was applied to the obverse surface of a kraft paper having a basis weight of 100 g/m² and then a non-woven fabric of polypropylene was superposed on the coated surface of the kraft paper and the resultant composite was dried. Then, a polyacrylic ester type tackiness agent was applied to the reverse surface of the kraft paper and a release paper was attached fast to the layer of the tackiness agent to obtain a tape of lubricating material (1) for the extraction of a temporarily buried reinforcement to be used as a control. This tape had a thickness of 400 µm.

Then, this lubricating material (1) for control was applied fast to the obverse surface of a planar iron sheet 150 mm in height and 70 mm in width.

The planar iron sheet having the lubricating material (1) for control applied fast thereto was placed in a container filled with cement milk obtained by blending cement, water, bentonite, and earth. The planar iron sheet wrapped with the lubricating material (1) for control, after 3 months' standing in the cement, was tested for the strength required for the extraction thereof from the cement.

The planar iron sheet coated with the lubricating material (1) for control could be extracted with a force of 70 g/cm². The work of applying the lubricating material (1) for control fast to the planar iron sheet was troublesome. When the planar iron sheet was extracted from the cement, the used lubricating material (1) for control was still adhering to the surface of the extracted planar iron sheet. For the purpose of putting this extracted planar iron sheet to use again, it was necessary to strip it of the adhering lubricating material (1) for control. It was not in a state to be directly put to use again as a reinforcement.

### Control 2

A surface-treating agent composed of 15 parts by weight of a water-absorbent polymer, 35 parts by weight of an extender of an acrylic type resin, 25 parts by weight of xylene, 5 parts by weight of n-butanol, and 20 parts by weight of methylethyl ketone was applied to a planar iron sheet 150 mm in height and 70 mm in width. The applied layer of the surface-treating agent was dried. Then, the coated planar iron sheet was placed in a container filled with cement milk obtained by blending cement, water, bentonite, and earth. The planar iron sheet coated with the surface-treating agent, after three months' standing in the cement, was tested for the strength required for the extraction thereof from the cement.

The planar iron sheet coated with the surface-treating agent could be extracted with a force of 50 g/cm². The application of the surface-treating agent to the planar iron sheet was a troublesome work. The planar iron sheet thus extracted was in such a state that the water-absorbent polymer and the extender were still adhering to the surface thereof. For the purpose of putting this extracted planar iron sheet to use again, it was necessary to strip it of the adhering substances. It was not in a state to be directly put to use again as a reinforcement.

### Control 3

A planar iron sheet 150 mm in height and 70 mm in width was placed alone as a temporary reinforcement in a container filled with cement milk obtained by blending cement, water, bentonite, and earth. An attempt to extract this planar iron sheet from the cement after its 3 months' standing in the cement entailed difficulty.

### Example 4

An aqueous 40 wt% monomer solution was produced by preparing an aqueous solution of sodium acrylate having a 60% portion thereof neutralized with sodium hydroxide and dissolving 0.1 mol% of methylenebisacrylamide (based on the amount of the sodium acrylate monomer) and 1.0 g/mol of sodium persulfate (based on the amount of the sodium acrylate monomer) in the aqueous sodium acrylate solution. A non-woven fabric made of complex fibers of polyethylenepolypropylene and having a basis weight of 25 g/m² was immersed in the aqueous monomer solution and impregnated with this solution and then wrung with rollers to remove excess aqueous monomer solution and effect deposition of the aqueous monomer solution on the non-woven fabric at a ratio of 180 g/m². The impregnated non-woven fabric was heated to effect radical polymerization of the monomer solution in the fabric and obtain a water-absorbent polymer sheet (3) having a water-absorbent polymer directly fixed at a ratio of 40 g/m² in the fabric. This sheet was capable of absorbing 80 times its weight of purified water. This water-absorbent polymer sheet (3) was labeled "a lubricating material (4) of this invention for the extraction of a temporarily buried reinforcement." It had a thickness of 250 µm.

This lubricating material (4) for the extraction of the temporarily buried reinforcement was folded and the opposite ends of the folded material were heat sealed to obtain a tube about 20 cm in diameter. The end part of this tube was heat sealed to produce a bag 20 cm in diameter and 30 cm in length. A steel H pile 3 cm in width and 30 cm in length was inserted into this bag.

Subsequently, the steel H pile placed in the bag of the lubricating material (4) for the extraction of the temporarily buried reinforcement was placed in a container made of polypropylene and measuring 9 cm in diameter and 27 cm in height and filled with soil cement. The soil cement was prepared by blending 12.8 parts by weight of cement, 52.6 parts by weight of water, 1.3 parts by weight of bentonite, and 33.9 parts by weight of clay.

After the steel H pile had stood in the cement for 30 days, it could be extracted from the hardened cement with a maximum load of 20 kgf.

### Example 5

A water-impermeable polypropylene layer 20 µm in thickness was formed on one side of the water-absorbent polymer sheet (3) obtained in Example 5 by melt extruding polypropylene and applying the extruded molten polymer to the one side of the water-absorbent polymer sheet (3). Thus, a lubricating material (5) of this invention for the extraction of a temporarily buried reinforcement was obtained.

A steel H pile was placed in the lubricating material (5) and placed in soil cement in the same manner as in Example 4.

After the steel H pile had stood in the cement for 30 days, it could be extracted from the hardened cement with a maximum load of 11 kgf. The surface of the extracted steel H pile showed absolutely no sign of either residual cement or rusting.

### Example 6

A water-impermeable polypropylene layer 100 µm in thickness was formed on one side of the water-absorbent polymer sheet (3) obtained in Example 5 by melt extruding polypropylene and applying the extruded molten polymer to the one side of the water-absorbent polymer sheet (3). Thus, a lubricating material (6) of this invention for the extraction of a temporarily buried reinforcement was obtained.

A steel H pile was placed in the lubricating material (6) and placed in soil cement in the same manner as in Example 4.

After the steel H pile had stood in the cement for 30 days, it could be extracted from the hardened cement with a maximum load of 1 kgf. The surface of the extracted steel H pile showed absolutely no sign of either residual cement or rusting.

### Control 4

An H bar was placed in soil cement by following the procedure of Example 4 while omitting the deposition of a lubricating material for the extraction of a temporarily buried reinforcement.

After the steel H pile had stood in the cement for 30 days, it could be extracted from the hardened cement with a maximum load of 13 kgf. The surface of the extracted steel H pile showed a sign of both residual cement and rusting.

### Control 5

The procedure of Example 4 was repeated excepting a steel H pile inserted in a bag 100 µm in thickness was placed in cement.

After the steel H pile had stood in the cement for 30 days, it could be extracted from the hardened cement with a maximum load of 10 kgf.

### Example 7

The lubricating material (5) obtained in Example 5 for the extraction of a temporarily buried reinforcement was folded with the polypropylene layer held on the inner side and the joined edges of the folded material were heat sealed. The folded material was cut into lengths of 6 m. Each cut length of the folded material was fabricated into an envelope 6 m in length and 1 m in width by heat sealing one cut end of the length. The envelope was corrugated by inserting alternating folds at intervals of 50 cm to acquire the shape of bellows.

Subsequently, the lubricating material (5) so fabricated in the shape of a bellows was set in place on a supporting base as shown in Fig. 3. A steel H pile 5 m in length and 20 cm in width suspended from above by a crane was inserted into the bag and buried in a hole 60 cm in diameter and 5 m in depth filled with soil cement. This soil cement was composed of 280 parts by weight of cement, 25 parts by weight of bentonite, and 900 parts by weight of water.

After the steel H pile had stood in the soil cement for one month, it could be extracted from the hardened cement with a maximum load of 1.4 tons. The surface of the extracted steel H pile showed no sign of either residual cement or rusting. Thus, the steel H pile was in a state to be directly put to use again.

In the case of an H bar which was directly buried for the purpose of comparison in the soil cement in the same manner as described above, a maximum load of 21 tons was required for extracting the steel H pile from the hardened cement. The periphery of the extracted steel H pile showed a sign of both residual cement and rusting.

### Example 8

The procedure of Example 7 was repeated while using a hole 10 m in depth and a steel H pile 10 m in length and 30 cm in width instead. The lubricating material (5) fabricated in the shape of a bellows for the extraction of a temporarily buried reinforcement had a length of 11 m.

When the steel H pile was extracted from the hardened soil cement after it had stood in the hole for three months, the maximum load required for the extraction was 2 tons. The surface of the extracted steel H pile showed no sign of either residual cement or rusting. The extracted steel H pile was in such a state as to be directly put to use again.

In the case of a steel H pile which was directly buried for the purpose of comparison in the soil cement in the same manner as described above, a load exceeding 100 tons failed to extract the steel H pile from the cement.

## Claims

1. A lubricating material for the extraction of a temporarily buried reinforcement, characterized by being provided with a water-absorbent polymer sheet layer having a water-absorbent polymer directly fixed on a substrate.

2. A lubricating material according to claim 1, wherein said water-absorbent polymer sheet has been obtained by polymerizing on said substrate a water-soluble ethylenically unsaturated monomer capable of being converted by polymerization into a water-absorbent polymer.

3. A lubricating material according to claim 1 or claim 2, wherein said substrate is a porous substance.

4. A lubricating material according to any of claims 1 to 3, wherein the amount of said water-absorbent polymer is in the range of from 10 to 1000 parts by weight, based on 100 parts by weight of said substrate.

5. A lubricating material according to claim 3, wherein said porous substance is a fibrous substance or a sponge.

6. A lubricating material according to any of claims 1 to 5, wherein a thickness of said lubricating material is in the range of from 10 to 1000 µm.

7. A lubricating material according to any of claims 1 to 6, wherein said water-absorbent polymer has been obtained by polymerizing a monomer having as a main component thereof at least one water-soluble ethylenically unsaturated monomer selected from the group consisting of (meth)acrylic acid, (meth)acryic acid salts, sulfonic acid group-containing acrylic esters and salts thereof, and 2-(meth)acrylamide-2-methylpropane sulfonic acid and salts thereof.

8. A lubricating material according to claim 7, wherein said water-absorbent polymer contains a sulfonic acid group.

9. A lubricating material according to claim 7 or claim 8, wherein said water-soluble ethylenically unsaturated monomer contains a cross-linking agent in an amount in the range of from 0.001 to 10 mol%, based on the amount of said monomer.

10. A lubricating material according to any of claims 1 to 9, wherein a water-impermeable layer is disposed on one side of said water-absorbent polymer sheet layer.

11. A lubricating material according to claim 10, wherein a thickness of said water-impermeable layer is in the range of 1 to 1000 µm.

12. A lubricating material according to any of claims 1 to 11, wherein said lubricating material is in the shape of a bag or a tube.

13. A lubricating material according to claim 12, wherein a water-impermeable layer is provided on the inner side of said water-absorbent polymer layer of said lubricating material in the shape of a bag or a tube.

14. A lubricating material according to claim 12 or claim 13, wherein a hanger is attached to an opening end of said bag or said tube.
